

Aug. 17, 1926.

1,596,640

L. VON REIS

METHOD AND PLANT FOR MANUFACTURING PLATE GLASS

Filed April 28, 1926

FIG. 1.



FIG. 2.



FIG. 3.



Inventor:

Lambert von Reis

per.  
J. J. Lawrence  
Attorney.

## UNITED STATES PATENT OFFICE.

LAMBERT VON REIS, OF HERZOGENRATH, GERMANY.

## METHOD AND PLANT FOR MANUFACTURING PLATE GLASS.

Application filed April 28, 1926, Serial No. 105,319, and in Germany May 4, 1925.

In the manufacture of plate glass on glass rolling machines the plates when rolled out have to be carried as quickly as possible into the annealing kiln in order to prevent them from warping or cracking because of being excessively cooled down by remaining too long in the atmosphere or in contact with the tables designed to receive the rolled plates and convey them to the said kiln. To this end, it has hitherto been customary to carry the plate immediately after or even during the rolling on a conveying table to the opening of the annealing kiln and shifting it into the kiln as soon as this can be done without affecting the consistency of the plate. If comparatively small glass plates are made, this known method can be applied without any danger for the plates. However, this method encounters serious difficulties in the manufacture of particularly large plates such as of plates made each from the whole contents of a large melting pot. Before the plates can be introduced into the annealing kiln the part of such large plates rolled out first is already relatively cold, while the intermediate or last part is still very hot. It is therefore necessary to delay the shifting of such a plate into the annealing kiln until the intermediate and rear parts have also become so hard that the plate can stand the shifting into the kiln. Owing to the large size of the plate it has, however, occurred that the part rolled out first had already warped or cracked before the intermediate and last part had attained the hardness required for the introduction into the kiln. In such cases, the plates therefore become wholly or partly useless. With a view of remedying this drawback, it has been proposed to seize the plate at its fore-end, which of course solidifies first, and to shift it in this way into the kiln. But in this case, it is necessary to leave the plate on its first place in the annealing kiln for a relatively long time in order to subject it to a heat interchange in all its parts and remove the stresses still prevailing in it. It has further been proposed to protect the plates against the influence of the atmosphere by conveying them through conduits and preventing in this way an excessive cooling down of the plates during their travel to the annealing kiln. These conduits are, however, very expensive and impedimental in service and besides have the disadvantage of rendering it

impossible to satisfactorily watch the glass so that severe losses are liable to be entailed.

Now, the invention has for its object to devise a method by which the said disadvantages are avoided in a simple and efficient manner. This method consists in maintaining the glass plates on their way from the glass rolling machine to the annealing kiln at an almost uniform temperature in all their parts by partly cooling or heating the plates. According to the prevailing circumstances, the plates are only partly cooled or only partly heated or they are partly cooled and partly heated at the same time.

For carrying out the method, the portable receiving and conveying table for the glass plates made on the glass rolling machine is, for instance, provided with means for heating a certain part of the table. Thus, the foremost third part of the table, i. e. the end of the table which receives the part of the plate rolled out first, may have mounted in it a heating device which heats the table surface from within and therefore keeps the part of the plate rolled out first so warm that a too rapid cooling down of that plate part and the consequent disadvantages are avoided. The heating of the table may be effected by means of electric current, gas, steam, coal, coke or the like. For obtaining a heat interchange in all parts of the plate, there may be used in combination with the heating device in the fore-end of the table a cooling device which consists, for instance, of one or more air blowers or similar means designed to act from above on the intermediate or rearmost part of the glass plates which is still very hot immediately after it has been rolled out. As a result of the heating of the forepart and simultaneous cooling of the rear part a rapid heat interchange is attained. The blowers may have different powers so as to act with different intensities on the plates as may sometimes be desirable. The action of the heating device in the foremost table part and the admission of air on the intermediate and rearmost table parts may be regulated in such a manner as to make the plate in all its parts free from stresses during its travel to and before its introduction into the annealing kiln. The plate treated according to the invention can also be shifted into the kiln sooner than in the old methods.

Another advantage of the invention over

the known methods resides in that the annealing kilns and the rolling machine may be arranged at any place and at any desired distance from one another, because with 5 the conveying tables constructed according to the invention the glass plates can be carried for larger distances than has hitherto been possible.

The accompanying drawing illustrates, 10 by way of example, some devices for carrying out the new method.

Fig. 1 is a side elevation, partly in section, of a glass rolling machine and a conveying table provided in its fore-part with 15 an electric heating device;

Fig. 2 is a side elevation of a similar device including a conveying table and a large blower arranged above the rear part of the table;

20 Fig. 3 is a similar side elevation illustrating two conveying tables provided in the fore-part with a coal furnace and one having arranged above its rear part three blowers of different powers.

25 Referring first to Fig. 1, *a* designates a glass rolling machine, *b* is a receiving and conveying table for the glass plates rolled out by the machine, *c* is an electric heating device mounted in the fore-part of the 30 table, and *d* are contacts adapted to connect the heating device *c* with the current lines *e*. At the proper time, the fore-part of the table is heated by means of the heating device *c* to a suitable temperature, thereby 35 preventing the fore-end of the rolled glass plate from cooling down too quickly and rendering it possible to introduce the plate into the annealing kiln in a condition in which all parts of the plate have the same 40 temperature.

According to Fig. 2 an air blower *f* is arranged above the receiving and conveying table *b*. This blower serves to blow air on the rear part of the plate, which when leaving the rolling machine *a* is always hotter than the fore-part of the plate, and to cool the rear part down to a temperature corresponding to the temperature of the fore-part.

45 Fig. 3 shows the combination of the devices according to Figs. 1 and 2. The arrangement is, for instance, so that the foremost third of the plate is heated by the de-

vice *c*, while the two last thirds of the plate are cooled by means of air blown on them by 55 air nozzles *i*, *h* and *g* which are of powers gradually increasing toward the rear end of the plate. In this case a very quick heat interchange throughout the whole glass plate is attained.

60 Having thus described my invention, what I claim as new and desire to secure by Letters-Patent is:—

1. The method of manufacturing plate glass, which consists in rolling the glass 65 plates on a rolling machine, carrying the rolled glass plates from the rolling machine to an annealing kiln, and while on their way to this kiln heating that part of the plates which has been rolled out first. 70

2. The method of manufacturing plate glass, which consists in rolling the glass 75 plates on a rolling machine, carrying the rolled glass plates from the rolling machine to an annealing kiln, and while on their way to this kiln cooling that part of the plates which has been rolled out last.

3. The method of manufacturing plate glass, which consists in rolling the glass 80 plates on a rolling machine, carrying the rolled glass plates from the rolling machine to an annealing kiln, and while on their way to this kiln heating the fore-part and simultaneously cooling the rear part of the plates. 85

4. In a plant for manufacturing plate glass, comprising a rolling machine, traveling tables for receiving the rolled glass plates and carrying them to an annealing kiln, and means for heating the fore-part of the tables. 90

5. In a plant for manufacturing plate glass, comprising a rolling machine, traveling tables for receiving the rolled glass plates and carrying them to an annealing kiln, and means for cooling the rear part of the tables. 95

6. In a plant for manufacturing plate glass, comprising a rolling machine, traveling tables for receiving the rolled glass plates and carrying them to an annealing kiln, and means for heating the fore-part and simultaneously cooling the rear part of the tables. 100

In testimony whereof I have signed my name to this specification.

LAMBERT von REIS.